

Feb. 8, 1938.

J. LITHGOW

2,108,017

METHOD OF COATING CONTAINERS

Filed Feb. 27, 1936

2 Sheets-Sheet 1



Fig. 2.

James *Inventor*,  
Lithgow  
By: Glenn S. Noble *Attty.*

Feb. 8, 1938.

J. LITHGOW

2,108,017

METHOD OF COATING CONTAINERS

Filed Feb. 27, 1936

2 Sheets-Sheet 2



James *Inventor*  
Lithgow

By: Glenn S. Noble *Atty.*

## UNITED STATES PATENT OFFICE

2,108,017

## METHOD OF COATING CONTAINERS

James Lithgow, Chicago, Ill., assignor to Lithgow Corporation, Chicago, Ill., a corporation of Delaware

Application February 27, 1936, Serial No. 65,978

6 Claims. (Cl. 91—70)

This invention relates to the coating or lining of metal containers or tanks for the purpose of protecting the contents thereof or preventing the contents from coming in contact with the metal 5 of the container and is particularly directed to large tanks such as tank cars, and tanks mounted in position for permanent installation as in breweries, factories, or the like.

Heretofore several methods have been used or 10 proposed for lining such tanks or containers. One of these methods contemplates the use of glass or vitreous enamel which can only be applied at the factory where the container is made and requires high temperatures or around 1700° 15 Fahrenheit to apply the same. Another method consists in the relatively cold application of pitch or base coatings in which small sections of the surface of the container are treated at a time. Another method contemplates spraying non- 20 ferrous metals on the inner surface but all of these different processes have been found objectionable for various reasons which are familiar to those having to do with this art.

In accordance with the present invention I 25 provide a novel method of coating or lining containers of the character indicated whereby the contents such as various foods, drinks, or bulk liquids may be maintained in a sterile condition and will be protected from contamination or dis- 30 coloration through contact with the material of the container. My improved process involves the use of a suitable lining material such as low temperature baking enamel or lacquer which is inert, when properly cured or baked, to food products 35 or other contents to be placed or kept in the container. There are a large variety of types or kinds of paints, enamels or lacquers which are adapted to be used for the present purposes to meet the particular conditions as respect to the 40 food or materials to be placed in the container and the present invention contemplates the use of any suitable coating material which may be adapted for the particular use for which the tank or container is intended.

45 The principal object of the present invention is to provide a method of lining or coating containers, tanks, or the like, particularly after the same have been mounted or installed in operating position or mounted in position for permanent installation, by applying the coating material and then subjecting the same to heat introduced into the container for curing and baking the coating material on the surface.

50 Other advantages and objects will appear more particularly from the following description taken

in connection with the accompanying drawings in which

Figure 1 is a longitudinal sectional view of a tank car illustrating an application of my improved method;

Figure 2 is a cross sectional view of the same showing the heating apparatus;

Figure 3 is a longitudinal sectional view illustrating any ordinary or preferred form of processing tank which is being lined or coated;

Figure 4 is a vertical sectional view of a slightly modified form of upright tank illustrating the lining method; and

Figure 5 is a vertical sectional view showing the arrangement for lining the metal base or bottom 15 of a wooden tank.

In carrying out this invention the container such as the container 6 of the tank car illustrated in Figure 1, is thoroughly cleaned and the inner surface sand blasted preparatory to receiving the coating or lining 7 on material which is capable of being hardened by baking at a relatively low temperature, such as paint, enamel or lacquer which may be applied in any suitable manner but preferably by means of a brush. This coating will ordinarily be allowed to air dry for about three hours or more and is then baked on in accordance with my improved system. Any number of coats may then be applied and baked on in accordance with the following method but 20 it will only be necessary to describe the operation for the first coat.

The tank which will ordinarily be made of steel or similar metal is enclosed or covered with a sectional insulating blanket 8 of any suitable material such as mineral wool, or other material which will lend itself to being formed into portable sections so that they may be transferred from tank to tank and connected together in any suitable manner or fastened onto the outer surface of the tank to suit the various sizes and shapes thereof.

It is necessary or desirable to be able to determine the temperature of the metal of all parts of the tank or container which is being treated 45 which may be done by any suitable temperature measuring apparatus such as thermometers, pyrometers, or the like. As a convenient method of determining the temperatures at different parts of the tank I provide wires or thermo-couples such as shown at 9 which are suitably connected with the tank and which may lead to the measuring instrument such as a portable potentiometer, thermostat, pyrometer or the like. These wires are preferably arranged so that the dif- 50 55

ferent pairs may be conveniently connected and disconnected with the instrument so that any desired number of temperature reading may be made for the different portions of the container.

5 It is necessary to determine the temperature of the metal of the container as the bonding of the coating to the inner surface of the metal is quite critical as respects to the temperature. If the temperature is too low the lacquer or coating will

10 not be properly cured and baked and if the temperature becomes too high the coating is apt to become brittle. It is necessary to take the temperatures of the metal at various points throughout the tank or container in order to

15 have all parts thereof heated to the proper degree. This will be more readily understood when it is considered that tank cars which I have treated in accordance with this method are approximately seven feet in diameter and thirty-

20 two to thirty-eight feet long. Storage or other tanks which I have lined in accordance with this process have been upwards of twelve feet in diameter and seventy feet long. The tendency of heat is to rise and accordingly it is necessary to

25 provide means for properly determining the temperature at different portions of the tank and particularly along the bottom in order to insure proper curing and baking of the coating throughout the interior surface.

30 The heat for baking may be derived from any suitable source but I have shown a portable furnace or heater 11 which may be heated by the combustion of gas, oil, solid fuel, or the like. The furnace is directly connected to a fan 12 which is

35 driven by a motor 13 which may be of the variable type in order to regulate the air supply. A conduit or pipe 14 leads from the furnace into the tank or container 6 where it is provided with discharge means for equalizing the distribution

40 of the hot air throughout the container. As shown in Figure 1 the pipe 14 has two lateral discharge branches 15 directed toward the ends of the tank and a down discharge branch 16 directed toward the bottom and outlet 17 of the tank.

45 These outlets are preferably provided with screens 18 to prevent any objectionable particles being blown into the container. After the heating apparatus has been arranged as shown the curing and baking are accomplished by blowing a

50 sufficient volume of hot air or gas into the tank to reach all interior surfaces and to raise the temperature to any desired degree. For instance with some lacquers the temperature is gradually raised for three or four hours until the temperature

55 of the metal of the container reaches approximately 250° F. to 275° F. and the temperature is held at this point for about one hour. Of course the time and amount of heat will be dependent upon the character of the coating

60 material as above suggested. The hot air or gases forced into the container from the furnace 11 are permitted to escape through any suitable openings in the container and as shown in Figure 1 the outlet pipe or connection 17 which is also

65 lined or coated will serve as an escape and at the same time will become sufficiently heated to bake the lacquer applied therein. The distribution of the air throughout the tank may also be controlled by arranging the outlet openings in order

70 to suit the type or shape of the tank. After the desired number of coatings have been applied the heating equipment may be removed and the tank will be in condition for use. The sectional or

75 removable insulation 8 and the portable heating

apparatus may be readily moved from one tank to another as will be readily understood.

The tank 19 shown in Figure 3 may represent a horizontal type of container intended for industrial purposes which is shown with a coating 5 20. The inlet pipe 21 for conducting heat from the furnace or source of heat supply is preferably stepped down or reduced in diameter to provide sections 22 and 23 and this discharge portion is provided with holes 24 which are arranged along 10 the same as indicated in order to direct the heat or hot air to the different portions of the tank. The pipe 21 may be supported in the tank by means of hangers or supports 25 or in any other suitable manner. In this arrangement the tank 15 is also provided with temperature measuring means or thermo-couples the same as in the form shown in Figure 1.

The upright tank 26 shown in Figure 4 is provided with a lacquer lining 27 which is applied 20 as above described. In this instance the inlet pipe 28 has a vertical branch 29 with holes 30 in the sides thereof. The upper end of the branch 29 may be provided with a deflector 31 and a hole or opening left in the lower end, the entire arrangement being such that the heat will be spread uniformly throughout the tank in order to give an even or uniform baking of the coating throughout the tank.

Figure 5 shows a tank 32 having an upper portion made of wood and a bottom or base 33 formed of metal such as cast iron, which type of tank is in more or less common use. While it is not necessary to coat the main part of the tank it is desirable to coat or line the bottom 33 with a lining 34 as shown. The heat is introduced as above described through a pipe 35 from any suitable source of heat supply, this pipe being conveniently introduced at the bottom and provided at its upper end with a deflector 36 for distributing the 40 gases which escape through openings 37. In order to confine the lining to the cast iron or metal bottom I provide a floor or partition 38 which is arranged above the upper end of the bottom and which has a lower insulating surface 39 for retaining the heat. This partition is preferably made in sections for easy insertion and so that it may be used for different tanks if desired.

The application of the heat to these different forms of tanks will be apparent from the above 50 description. The amount of heat and regulation thereof may be controlled in any well known manner as by regulating the amount of fuel supplied to the furnace or heater and by varying the speed of the fan motor and the heat supplied to different portions of the tank may be regulated by moving the inlet pipes or changing the outlet openings. After the one or several layers of lacquer or coating have been applied and baked on, the heat conducting and distributing devices and 60 the temperature measuring apparatus and other parts may be removed and the tank or container will be ready for use.

In the actual application of this invention for commercial purposes I have found that by using 65 a lacquer which can be applied at room temperatures a perfect bond will be made with the steel and an even coat provided over all surfaces. My improved method of baking provides full temperature control at all times, thereby insuring the 70 baking of the entire lining to a uniform hardness and eliminating the possibility of soft spots which would permit oxidation of the steel and result in flaking off of the lining. By using comparatively low temperatures I am able to bake vessels 75

of irregular shape without distortion and can also operate on tanks in places such as brewery cellars which must be maintained at temperatures not over 40° F. without interfering with the regular plant operation. This process also provides means for recoating or lining old tanks which would otherwise have to be replaced at great expense and with resulting loss of operation while the tanks were transferred and which might also require the demolition of building walls to permit exit and entry of the tanks. The use of my method for lining the bottom cones or bases of wooden tanks is also highly desirable as it may be done without injury to the wooden staves and this fills a long felt want of several chemical industries in which products are handled which affect metal but which nevertheless require the use of metal bottoms in order to make the necessary pipe connections.

While I have outlined various uses and advantages of my invention it may also be applicable to other containers and other advantages may be apparent to those familiar with the art. Any invention or subject matter herein shown and described but not claimed, is not intended to be dedicated to the public, insofar as such subject matter is shown, described and claimed in my pending application for Metal coating, filed December 2, 1937, Serial No. 177,781. Accordingly I do not wish to limit my claims to the particular method or apparatus herein shown or described except as specified in the following claims in which I claim.

1. The method of lining a metal tank which comprises first covering the tank with a covering of heat insulating material, then coating the inner surface of the tank with a suitable coating material which is adapted to be baked on, permitting said coating material to air dry, then introducing a conduit into the tank and forcing gases heated to the necessary temperature for baking the coating material, after it has become dry, through the conduit into the tank for a sufficient length of time to bake the coating to a uniform hardness, said gases being permitted to escape from the tank as the baking progresses.

2. The process of coating relatively large metal tanks mounted in position for permanent insulation, which comprises applying a lining of a material which is capable of being baked at a relatively low temperature to harden the same, then providing a portable furnace having a pipe adapted to lead therefrom into the container and having means for blowing air therethrough, then driving the heated air through said pipe into the container for a sufficient length of time to bake the lining applied thereto to obtain a lining of uniform hardness.

3. The process of coating the interiors of relatively large metal tanks mounted in position for permanent installation, which includes placing a

covering of heat insulating material around the tank, applying a coating to the inside of the tank, which coating is capable of being baked at a relatively low temperature, providing a portable furnace having a power driven fan for driving air therethrough, connecting the furnace with the tank and forcing gases heated to approximately 250° F. to 275° F. into the tank for a sufficient length of time to properly harden the lining previously applied thereto and finally permitting the tank to cool.

4. The method of coating the metal portion of a tank, which comprises closing off said metal portion from the remainder of the tank, then painting the inner surface of said portion with a material which is capable of being hardened by baking at a relatively low temperature, temporarily covering the exposed outer surfaces of said portion with insulating material to be kept thereon during the baking process only, then directing gases which are heated to a baking temperature into said portion, said gases being directed into said portion a sufficient length of time to bake said material to a uniform hardness, and finally removing the insulation from said portion.

5. The herein described method of applying durable and substantially permanent linings to large metal tanks, metal tank cars, or the like, which comprises covering the tank temporarily with insulating material to prevent loss of heat during the baking operation, then coating the inner surface of the tank with a suitable lining material which is capable of being hardened by baking at a relatively low temperature, allowing said lining to dry, then directing into the tank, gases which are heated sufficiently to harden the lining material, and finally removing the insulating material, leaving said tank with a suitably hardened lining as and for the purposes described.

6. The herein described method of protecting the interiors of metal containers of large size from the action of material placed therein, which comprises covering the container with a heat insulating cover, cleaning the inner surfaces of the container by sand-blasting, then applying a layer of coating material in liquid form, which material is of a nature that it may be hardened to the desired consistency by baking, allowing the layer to air dry until thoroughly dried, then forcing heated gases under pressure into the container and gradually raising the temperature of the metal of the container until it reaches approximately 250° F. to 275° F. and holding the temperature at approximately this heat until the layer is sufficiently hardened, then permitting the tank to cool, and removing the insulation from the outer surface thereof.

JAMES LITHGOW. 60